

F. W. HAWKINS & G. F. KEY.

PROCESS OF REFINING IRON.

APPLICATION FILED MAY 21, 1906.

949,474.

Patented Feb. 15, 1910.



WITNESSES

*Geo. H. Graves*

James O. Barry, Esq.

INVENTORS  
FREDERICK W. HAWKINS  
GEORGE F. KEY.

*Whittemore, Hubbell & Whittemore*  
ATTYS.

# UNITED STATES PATENT OFFICE.

FREDERICK W. HAWKINS AND GEORGE F. KEY, OF DETROIT, MICHIGAN, ASSIGNEES  
TO THE GLOBE STEEL FILTRATION PROCESS COMPANY, OF DETROIT, MICHIGAN, A  
CORPORATION OF ARIZONA TERRITORY.

## PROCESS OF REFINING IRON.

949,474.

Specification of Letters Patent. Patented Feb. 15, 1910.

Application filed May 21, 1906. Serial No. 318,053.

To all whom it may concern:

Be it known that we, FREDERICK W. HAWKINS and GEORGE F. KEY, citizens of the United States of America, residing at 5 Detroit, in the county of Wayne and State of Michigan, have invented certain new and useful Improvements in Processes of Refining Iron, of which the following is a specification, reference being had therein to 10 the accompanying drawings.

The invention relates to the art of refining iron and has for its object the obtaining of a process in which the metal receives a uniform treatment through its mass.

15 It is a further object to reduce the time necessary for completing the refining.

In the drawing, an apparatus is illustrated 20 diagrammatically in longitudinal section, in which our improved process may be carried out.

It is a special object of our invention to 25 provide a process which is suitable for the refining of iron which, in its crude state, has a high percentage of impurities requiring for their elimination different treatment. For example, iron which contains both 30 silicon and phosphorus, or silicon, sulfur and phosphorus cannot be directly treated in an open-hearth basic-lined furnace, for the reason that the linings would be 35 destroyed by the reactions of the silicon. On the other hand, such metal cannot be refined by the Bessemer process, as this does not extract the phosphorus, and sulfur.

With our improved process the iron is 40 first treated in a receptacle or furnace herein referred to to eliminate the impurities which will yield to oxidation and subsequently, but in direct continuation of this first treatment, the metal is subjected to a second treatment, 45 with a basic material, in another furnace or chamber, which removes the phosphorus and sulfur. In the latter step and preferably in both steps of the process all portions of the metal are subjected to uniform treatment by atomizing or breaking up the molten mass into minute particles, this being 50 preferably accomplished by a blast of dry steam, or of dry steam and air, the latter being preferably pre-heated.

In the apparatus illustrated in the drawing, A is a preparatory furnace or reducing chamber, which is preferably mounted upon trunnions B upon a turntable C, so that

the furnace may be arranged either in a 55 horizontal position or in an inclined position for pouring out the molten metal. In this horizontal position one end of the chamber A is arranged in registration with a flue or stack connection D providing an escape 60 for the gases of combustion. The opposite end of the furnace is provided with a steam twyer E and one or more air twyers F, these twyers being arranged to direct their jets longitudinally of the furnace. G is a 65 well or receptacle formed in the upper wall of the furnace adjacent the end containing the twyers, said well terminating at its lower end in a slot or narrow passage. This well is adapted for the reception of the crude 70 molten metal which will pass through the narrow slot and will fall into the furnace A directly in the path of the jets issuing from the twyers E and F. E' are a series of twyers for blowing air over the molten metal 75 in the furnace A and assisting in oxidation. H is a second furnace which is arranged at a lower level than that of the furnace A and is stationary. This furnace H is also provided with steam and air twyers I and 80 J extending in through one of the end walls thereof to direct their jets longitudinally of the furnace. K is a metal well for the furnace H which also is provided with a narrow discharge opening for permitting metal in 85 the well to be discharged directly in the path of the jets from the twyers.

With the apparatus as described the refining process may be carried out as follows: A suitable quantity of the crude molten 90 metal is first poured into the well G while the furnace A is arranged in its horizontal position. At the same time air and steam, either in conjunction or separately, as conditions may require, are forced through the 95 twyers E and F so that metal dropping from the well may be blown into fine particles and scattered throughout the length of the furnace A. During the passage of the small particles of metal through the atmosphere within the furnace, a large percentage of the silicon, manganese and carbon will be removed by oxidation. The metal will then collect in the bottom of the furnace where it remains until the entire charge has passed 100 therein. The furnace A is then revolved on the turntable C and tilted upon the trunnions B so as to lower its open end over the

well K on the furnace H. This will permit the molten metal within the furnace A to be discharged into the well K from which it is fed through the restricted passage into the

5 path of the air and steam admitted through the twyters I and J. This will a second time atomize the molten metal with the result that the remainder of the silicon, manganese and carbon will be oxidized.

10 The bottom of the furnace H is covered with a layer of comminuted basic material which is heated to a high temperature by burning gases entering the furnace chamber from end ports L. This comminuted basic material forms a filter bed through which the minute particles of molten metal are obliged to percolate and in so doing the metal is brought into intimate contact with the basic material which extracts the phosphorus and sulfur. Thus the 15 metal which finally passes through the filter bed and collects in the bottom of the furnace H is purified both from silicon, manganese and carbon, and also from the phosphorus and sulfur.

20 The whole process may be carried out in a comparatively short period of time. By subjecting the molten metal to a second atomizing process all the oxidizable impurities are sufficiently eliminated before the 25 final treatment of percolation. At the same time the first atomizing of the metal will remove the larger part of the silicon and manganese and carbon so that the second treatment may be carried on in a basic lined 30 furnace without danger of injury to the linings.

35 In place of percolating the metal through a bed of comminuted basic material, this material may be infused in the molten metal as it is atomized the second time. We preferably, however, subject the metal to both 40 treatments, *i. e.*, a certain amount of comminuted basic material is infused in the molten metal while undergoing the second 45 atomizing process, and the scattered particles of metal are then percolated through the bed of comminuted basic material, as has been previously described.

50 The receptacle K of any desired construction has a vertical partition k dividing the same into a plurality of hoppers, the one constituting the hot well from which the molten metal issues through the restricted 55 outlet k', as above described, and the other a receptacle for the basic material K' to be infused in the molten metal.

What we claim is,—

1. The herein described process of refining iron which consists in first eliminating 60 a portion of the oxidizable impurities in the molten metal while in a divided state, by a process of oxidation, in then atomizing or breaking up the molten mass into minute 65 particles and scattering the same to com-

plete the oxidation, and then percolating the separate particles through a bed of comminuted material having a chemical affinity for the remaining impurities.

2. The herein described process of refining iron which consists in first subjecting the molten metal while in a divided state to a process of oxidation, whereby a portion of the oxidizable impurities is removed, in then atomizing or breaking up into minute 75 particles and scattering the partially purified molten metal to complete the oxidation of the oxidizable impurities and in finally percolating the particles through bed of a comminuted basic material. 80

3. The herein described process of refining iron which consists in first atomizing the molten metal in an oxidizing atmosphere, to remove a portion of the oxidizable impurities, and then re-atomizing the metal and scattering the particles over a bed of comminuted basic material whereby the remaining oxidizable impurities are first removed and other impurities are subsequently removed by percolation through the basic bed. 90

4. The herein described process of refining iron which consists in atomizing and re-atomizing the molten metal in successive treatments, and in scattering the separate particles through an oxidizing atmosphere 95 as herein described, and then passing the particles from the last atomizing treatment through a filter bed of comminuted basic material.

5. The herein-described process of refining 100 metal which consists in first eliminating a portion of the oxidizable impurities in the molten metal by a process of oxidation, and in subsequently atomizing the molten mass in an oxidizing atmosphere and treating the 105 same with comminuted basic material.

6. The herein-described process of refining metal which consists in first eliminating a portion of the oxidizable impurities in the molten metal by a process of oxidation, and 110 in subsequently infusing basic material into the molten mass in atomizing, and scattering the mass through an oxidizing atmosphere to complete the oxidation, and finally percolating the particles through a bed of 115 comminuted basic material.

7. The herein described process of refining metal, which consists in first introducing the molten metal into a furnace having a nonbasic lining and an oxidizing atmosphere, atomizing the metal as it enters the furnace whereby a portion of the oxidizable impurities is removed, in then introducing the partially purified molten metal into a second furnace having a basic lining and 120 an oxidizing atmosphere, atomizing or breaking up into minute particles and scattering the partially purified molten metal to complete the oxidation of the oxidizable impurities, and in finally percolating the 125 130

particles through a bed of comminuted basic material.

8. The herein described process of refining metal which consists in atomizing the 5 molten metal in a furnace having a non-basic lining and an oxidizing atmosphere whereby a portion of the oxidizable impurities in the molten metal is eliminated by oxidation, re-atomizing the metal and introducing it into a second furnace having a 10 basic lining and an oxidizing atmosphere, atomizing the partially purified molten

metal as it enters the furnace, and then passing the particles from the last atomizing treatment through a filter bed of commi- 15 nuted basic material.

In testimony whereof we affix our signatures in presence of two witnesses.

FREDERICK W. HAWKINS.  
GEORGE F. KEY.

Witnesses:

HARRY M. LAU,  
DAVID R. PERRY.